

2,393,821  
A method of preparing a photographic resist for use in the production of fine lines, such as cross hairs, scales, grati-  
cles, and the like, by exposing a photographic resist to light and then subjecting the exposed areas to a heat-  
carbonizing treatment.

# UNITED STATES PATENT OFFICE

Method and composition of producing fine lines photographically

André Schoen, Binghamton, N.Y., and Letha Lemon Patterson, Arlington, Va., assignors to General Aniline & Film Corporation, New York, N.Y., a corporation of Delaware

No Drawing. Application May 11, 1943.

Serial No. 486,544

This invention relates to the photographic reproduction of fine lines, such as the production of cross hairs used in gun sights and other observation instruments, as well as scales and grati-  
cles, and in general to designs in which very fine lines are desired. The invention also relates to compositions useful in the production of such fine lines, and in the preparation of resists for producing fine lines by etching.

In general the production of cross hairs, scales and other designs with very fine lines has heretofore been accomplished by the costly process of engraving with diamonds or other fine cutting tools. Attempts to produce such designs by a photographic process have proven to be unsatisfactory for a number of reasons, such as lack of resolution, poor adhesion of the lines to the surface material, lack of resistance to abrasion, and poor chemical resistance of the light-sensitive coating applied to the surface.

Thus, the U. S. Patent to Karl Gundlach, #1,922,434, granted on August 15, 1933, refers to the unsatisfactory results obtained by the prior methods utilized in producing fine lines of the nature above referred to. In referring to prior photomechanical methods of etching glass, the patentee states that while photomechanical methods of etching glass have already been suggested, these methods, which are in most cases based on the application of light-sensitive asphalt, or of chromate colloid layers, entailed great disadvantages and, therefore, hardly can be used in practice, the reason being that the light-sensitive layers are either not sensitive enough, as in the case of asphalt, or not resistant enough against the influence of hydrofluoric acid, as in the case of the chromate colloid layers.

It is accordingly an object of our invention to overcome the deficiencies of the prior art processes.

It is a further object of our invention to provide an effective, simple, inexpensive and practical means for producing fine lines of the nature above referred to on glass, metal and other surfaces. Copper has been found particularly suitable as a metal base.

It is a still further object of the invention to produce etched lines on the above mentioned bases.

In general, hydrofluoric acid and fluorides diffuse through all the photographic resists known to the art. This is recognized by Gundlach and to overcome this defect Gundlach found it necessary to utilize a metallic layer under the chromate layer in order to obtain fine lines photograph-

ically. We, however, have discovered that the light-sensitive colloidal chromate layers in which the colloid is fish glue, gelatin or casein can be rendered resistant to attack by hydrofluoric acid and its salts by treating the colloidal layer after exposure to a light image of the fine lines to be obtained with tannic acid-containing substance, and then subjecting the exposed areas to a heat-carbonizing treatment.

Our invention, therefore, consists in a method of producing fine lines photographically, which consists in exposing a photographic resist to light and then subjecting the exposed areas to a heat-carbonizing treatment.

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

5600

5605

5610

5615

5620

5625

5630

5635

5640

5645

5650

5655

5660

5665

5670

5675

5680

5685

5690

5695

5700

5705

5710

5715

5720

5725

5730

5735

5740

mixture is heated to the boiling point, for example, in a double boiler. When the albumen has completely coagulated and the solution cooled down to room temperature, it is filtered. The specific weight of the clear filtered solution is about 1.04. This solution is hereinbelow referred to as photo-engraver's glue solution.

An albumen solution comprising 20 gms. of dry albumen and 100 cc. of distilled water is prepared. The albumen is soaked in the water for about four hours and to the resulting solution is then added a small amount, for example, two drops of phenol or other suitable preservative. The solution is then filtered through cotton.

A solution comprising 4 gms. of ammonium bichromate and 100 cc. of distilled water is prepared.

A solution comprising 40 gms. of tannic acid and 100 cc. of distilled water is prepared by dissolving the tannic acid in the water with the aid of heat and then cooling to room temperature.

To prepare the sensitizing solution, three parts of the above prepared photoengraver's glue solution, one part of the albumen solution and one part of the ammonium bichromate solution are mixed thoroughly and then filtered, care being taken to carry out the mixing away from direct light and air as much as possible. However, conducting the preparation in a darkroom is not necessary.

A piece or plate of chemically cleaned and polished glass or other material on which the fine lines are to be produced is then coated with a thin coating of the sensitizing solution. Any well-known coating method may be utilized for this purpose, such as centrifugal coating, smear method, painting or other satisfactory coating procedure. The coated plate is then allowed to dry in the absence of extreme heat, direct sunlight and air currents, avoiding dust as much as possible. In this way, a light-sensitive chromate colloid layer is produced on the surface.

The scales or fine lines are obtained by exposing the sensitive layer to light through a fine line negative. For example, the exposure may be made through a contrasty negative of the fine lines to be obtained, using a 25 ampere arc lamp at two feet distance the exposure time being 2-3 minutes depending on the negative. This is only given as an example, and other times of exposure and types of exposure light may be utilized. To develop the image all that is necessary is to immerse the plate in a tepid water bath or wash under running water for five minutes. Care must be taken to insure that all unexposed sensitized material is washed away.

After developing, the plate is immersed for five minutes in the tannic acid solution. It is then again carefully washed, followed by a rinse in distilled water. The plate is then allowed to dry and the image is then heat-carbonized by exposing to heat until the maximum blackness of the image is obtained. Good results are obtained when an exposure at 450° F. for 30 minutes is utilized although other temperatures and periods of heating give equally good results. The fine lines so produced withstand the action of hydrofluoric acid and its salts. The lines also are resistant to abrasion and various solvents and cleaning fluids such as xylol. The lines show excellent resolution and the absence of graininess and roughness of edges common to prior methods of producing fine lines.

Although we prefer to use fish glue, gelatin

or casein may be utilized in the process in corresponding amounts. Likewise, instead of ammonium bichromate, there may be used potassium or sodium bichromate in equivalent amounts. The albumen may be omitted but improved results are obtained, particularly with respect to adhesion, when it is present in the light-sensitive layer.

The above embodiment of the process results in the production of fine lines and the products so obtained may be used directly as graticules, scales and cross hairs for technical and other purposes.

In the alternative embodiment, the fine lines are utilized as resists in the production of etched lines, scales and graticules on glass or on other inorganic bases such as copper. In photo-engraving and related processes where the image is etched into the base material, the chief problem is to find a resist which will withstand a certain amount of mechanical abrasion, adhere to the base and be impervious to the etching solution which is usually acidic in character. As pointed out above, some acids like hydrofluoric and its salts penetrate the usual photoengraving resists with ease and cannot be used when a photographic design has to be etched on glass. For this reason, the prior photoengraving resists cannot be used to produce fine lines by etching.

The prior art processes are unsatisfactory because in transferring very fine lines to glass or other base, the resist must of necessity be very thin in order to faithfully reproduce the fine details of the original which consists mostly of very fine lines, dashes or dots. Since the usual photoengraving resists are attacked by the acidic etching fluids, these fine lines are quickly attacked and the etched lines produced are not of high resolution but are ragged and not clearly defined.

For the production of fine lines, the resolving power of the light-sensitive coating must be extremely high to insure the faithful reproduction of microscopic detail. A photoengraving resist should preferably have a dark color which facilitates inspection prior to the application of the etching fluid.

In our alternative embodiment of producing fine lines, the same solutions and procedure are employed as in the first embodiment, except that for exposure, a contrasty positive is used to obtain a negative image of fine lines on the sensitized coating; that is, the image is washed away, leaving the surrounding area protected. Subsequent to the tannic acid treatment and carbonizing, the resist is dark in color which facilitates inspection and has great resistance to mechanical abrasion and to the selected etch. The plate is then treated with an appropriate etch which acts only in the area of the image, the resist, due to the tannic acid and subsequent baking treatment, possessing the novel property of withstanding the action of hydrofluoric acid and its salts. After the lines have been etched in the surface, the resist is then removed. The etched lines may then be filled in by use of any suitable black varnish.

By way of example, a more detailed description of this embodiment follows:

#### Example II

A glass plate chemically cleaned and polished is coated with the sensitizing solution prepared in the manner indicated in Example I. The coated plate is then exposed through a contrasty positive of the fine lines to be etched on the

glass base, and subsequently treated as in Example I with tannic acid, followed by heat-carbonization. The plate with the carbonized areas thereon acting as a resist is then treated with an etching solution of the following composition:

|                     |       |     |
|---------------------|-------|-----|
| Ammonium bifluoride | grams | 10  |
| Barium sulfate      | do    | 10  |
| Water               | cc    | 100 |

for a period of ten to fifteen seconds, although the time may be varied depending on the degree of etching desired.

The resist is then removed by immersing in a hot chromic acid solution. On the glass surface only the etched fine lines now remain. If a better visibility of the lines is desired, the etched lines may be filled in by the use of a suitable black varnish or any other suitable preparation.

The following is an example of the procedure as applied to the production of etched lines on a metal plate, such as copper:

*Example III*

The resist is prepared on a copper plate in the same manner as described in Example II above for its preparation on glass. The area of the image is then treated with a 35° Baumé solution of ferric chloride until the desired degree of etch is obtained. The resist is then removed by rubbing the plate with calcium carbonate.

In the above example of etching glass, any glass etching fluid may be utilized although the process is most effective with the use of ammonium bifluoride. However, hydrofluoric acid or any of its water soluble salts may also be used. Likewise, other etching fluids may be used for etching the copper or metal surfaces.

While several embodiments of the invention are herein described, it is to be understood that various modifications may be apparent to those skilled in the art without departing from the spirit and scope of this invention and we, therefore, do not wish to be limited by the precise details set forth, but desire to avail ourselves of such variations and modifications as come within the scope of the appended claims.

We claim:

1. A method of producing cross-hairs, graticules, scales and designs with fine lines on surfaces, which comprises coating a surface with a light-sensitive chromate colloid layer in which the colloid is selected from the group consisting of fish glue, casein and gelatin, exposing the layer to a light-projected image of fine lines, removing the unexposed areas of the layer, subjecting the exposed areas to a tannic acid-containing substance, and subjecting the tannic acid-treated areas of the layer to a heat-carbonizing treatment, whereby fine lines of high resistance to abrasion and chemical agencies, and high resolution, adhesion and density are obtained.

2. A process as in claim 1 in which the surface is glass.

3. A method of producing cross-hairs, graticules, scales and designs with fine lines on a glass surface which comprises coating a glass body with a light-sensitive solution composed of fish glue, albumen and ammonium bichromate, exposing the light-sensitive layer thus formed through a negative of the fine lines to be obtained, removing the unexposed areas of the layer by developing with water, subjecting the exposed areas of the layer to an aqueous solution of tannic acid, and subjecting the tannic acid

treated areas of the layer to a heat-carbonizing treatment until maximum blackness of the exposed areas is obtained, whereby fine lines of high resistance to abrasion and chemical agencies, and high resolution, adhesion and density are obtained.

4. A process as in claim 3 in which the carbonizing treatment is carried out by subjecting the tannic acid treated areas to a temperature of 10 about 450° F. for about thirty minutes.

5. A process for producing cross-hairs, graticules, scales and designs with fine lines on surfaces which comprises coating a surface with a light-sensitive chromate colloid layer in which the colloid is selected from the group consisting of fish glue, casein and gelatin, exposing the layer through a positive of the fine lines to be obtained, removing the unexposed areas of the layer, subjecting the exposed areas to a tannic acid-containing substance, subjecting the tannic acid-treated areas of the layer to a heat-carbonizing treatment, thereby converting the exposed areas into a resist, and subjecting to an etching solution those areas of the surface from 25 which the unexposed areas of the light-sensitive layer has been removed.

6. A process for producing cross-hairs, graticules, scale and designs with fine lines on glass surfaces which comprises coating a glass body

30 with a light-sensitive layer composed of an aqueous solution of ammonium bichromate, albumen and fish glue, exposing the layer through a positive of the fine lines to be obtained, washing out the unexposed areas of the layer with water, subjecting the exposed areas to an aqueous solution of tannic acid and subjecting the tannic acid treated areas of the layer to a heat-carbonizing treatment thereby converting the exposed areas into a resist, and subjecting to an aqueous etching solution composed of ammonium bifluoride and barium sulfate those areas of the glass surface from which the unexposed areas of the light-sensitive layer has been removed, and then removing the resist.

45 7. A process as in claim 6 in which the surface is composed of copper and in which the etching is carried out by means of an aqueous ferric chloride solution.

8. A composition for producing fine lines and 50 resists for etching of fine lines on surfaces which comprises the heat-carbonized reaction product of a tannic acid-treated, light-exposed mixture of a protein selected from the group consisting of fish glue, casein and gelatin, and a light-sensitive chromate, said composition being resistant to hydrofluoric acid and its salts.

9. A new resist for photoetching of fine lines 55 on surfaces comprising the heat-carbonized reaction product of a tannic acid-treated light-exposed mixture of fish glue, albumen and ammonium bichromate, said composition being resistant to hydrofluoric acid and its salts.

10. A composition for use in preparing a resist for photoetching of fine lines on surfaces comprising the reaction product of a protein selected from the group consisting of fish glue, gelatin and casein and a light-sensitive bichromate, said composition, on exposure to light and subsequent treatment with tannic acid followed by heat-carbonization, forming a resist which will withstand the action of hydrofluoric acid and its salts.

11. A body having on its surface fine lines, cross-hairs, scales and graticules composed of 75 the heat-carbonized reaction product of a tan-

nic acid-treated and light-exposed mixture of a protein selected from the group consisting of casein, gelatin and fish glue; and a light-sensitive chromate said reaction product being resistant to hydrofluoric acid and its salts.

12. A body having on its surface fine lines, cross-hairs, scales and graticules composed of

the heat-carbonized reaction product of a tannic acid-treated, light-exposed mixture of fish glue, albumen and ammonium bichromate said reaction product being resistant to hydrofluoric acid and its salts.

6

ANDRÉ SCHOEN.  
LETHA LEMON PATTERSON.